

April 28, 1953

P. W. BEAMER ET AL

2,636,219

METHOD OF PRODUCING SHOT

Filed Aug. 23, 1950

2 SHEETS—SHEET 1

Fig. 1.



WITNESSES:

*H. J. Basser*  
*R. W. Thomas*

INVENTORS

Paul W. Beamer and  
Wilson G. Young, Jr.

BY

*James W. Ely*  
ATTORNEY

April 28, 1953

P. W. BEAMER ET AL

2,636,219

## METHOD OF PRODUCING SHOT

Filed Aug. 23, 1950

2 SHEETS—SHEET 2

Fig.2.



Fig.3.



**WITNESSES:**

H. F. Sussner.  
D. W. Thomas

## INVENTORS

Paul W. Beamer and  
Wilson G. Young, Jr.

BY

BY  
*James H. Ely*  
ATTORNEY

## UNITED STATES PATENT OFFICE

2,636,219

## METHOD OF PRODUCING SHOT

Paul W. Beamer, Irwin, and Wilson G. Young, Jr.,  
Pittsburgh, Pa., assignors to Westinghouse  
Electric Corporation, East Pittsburgh, Pa., a  
corporation of Pennsylvania

Application August 23, 1950, Serial No. 180,974

3 Claims. (Cl. 18—47.3)

1

This invention relates to a method of producing melting stock and particularly to a method of producing melting stock in the form of metallic shot for use in precision casting.

Heretofore, melting stock for use in precision casting was produced by either pouring molten metal into core sand molds, thus forming cast pins, or by breaking up a stream of molten metal with a single jet of water so as to produce metallic shot. This latter method was carried out by first pouring molten metal contaminated with slag into an inclined V-shaped ceramic-lined trough. In order to remove the slag from the molten metal, a partition or dam was provided midway the length of the trough. The partition had an opening in the bottom thereof to allow the flow of the molten metal therethrough, the slag being retained in the trough by the dam. After passing through the opening in the partition, the molten metal continued to run down the inclined trough until it spilled over the end in the form of a stream of molten metal. This stream was then broken up by means of a single jet of water, thus producing the metallic shot.

These former methods of producing metallic shot, however, had several disadvantages. In the case of the cast pins formed by pouring the molten metal into the sand molds, the cost and time consumed in producing each pin were considerable. The other method in which metallic shot was produced had its disadvantages too. The size of the metallic shot produced by this latter method varied over wide limits, which was undesirable. The size of the shot produced ranged from extremely fine particles which would pass through a 20 mesh screen to very coarse particles which would not pass through a 2 mesh screen.

Where shot is used as the melting stock for the making of precision castings, the size of the shot is critical and must be closely controlled for best results. If it is too fine, its surface area is large with respect to the amount of metal of the shot which means that the amount of oxide on its surface for the given amount of metal is great. This is undesirable because the greater the amount of oxide per unit weight of metallic shot the greater is the amount of slag formed when the metal is remelted. The slag formed must be removed from the remelted material prior to its use in precision casting. If the metallic shot is too coarse, another problem arises since it will not pass through the mouth of a remelting furnace of the type used in melting stock for the making of precision castings. Therefore, un-

2

less the size of the metallic shot is proper, a great deal of the shot produced will have to be discarded.

Another disadvantage of the last-mentioned method in which metallic shot is produced is that the slag contaminates the ceramic-lined trough through which the metal runs with the result that the trough must be frequently replaced, causing time delays in the production of the shot as well as greatly adding to the cost thereof. The apparatus for carrying out the teachings of this invention is so constructed as to avoid this problem.

An object of this invention is the provision of a method for making metallic shot that is substantially spherical in shape and has a minimum of oxide on its surface.

Another object of this invention is to provide for subjecting a stream of molten metal to the action of a plurality of jets of water to impart a rotary motion to the metal and effectively break the stream into a plurality of substantially spherical shot.

Other objects of this invention will become apparent from the following description when taken in conjunction with the accompanying drawings, in which:

Figure 1 is an elevation view of the apparatus constructed in accordance with this invention;

Figure 2 is a detailed plan view of the shot ring shown in Figure 1; and

Figure 3 is a view in section taken along the line III—III of Figure 2 of the shot ring constructed in accordance with this invention.

Referring to Fig. 1 of the drawing, there is illustrated metallic shot-producing apparatus 3 for carrying out the teachings of this invention. As illustrated, the shot-producing apparatus 3 comprises a shot-making ring 10 disposed to receive molten metal 11 from a pouring receptacle 12 which is supplied from a melting furnace or reservoir 14 containing the molten metal 11, a tank 16 being positioned below the shot ring 10 for receiving the shot as will be described more fully hereinafter.

As illustrated, the pouring receptacle 12 is preferably a clay-graphite tundish having an opening 18 through the bottom for guiding the stream of molten metal 11 into the shot ring 10. The receptacle 12 is utilized to provide a constant supply of metal to the ring 10, such supply being controlled by maintaining the level of the molten metal 11 in the tundish at a predetermined height to maintain a predetermined pressure

head on the metal and thereby control the stream of metal.

The shot ring 10 comprises a cylinder 20 having several tiers of spaced passageways 22 extending through the cylinder wall in a predetermined direction to direct jets of water (to be described hereinafter). An annular chamber 24 is disposed around the cylindrical member 20 for containing a fluid, such as water 26, under pressure to feed it to the passageways 22. The chamber 24 comprises a ring-shaped channel member with the edges of the channel welded or brazed to the outer surface of the hollow cylindrical member 20 to form a closed conduit for the water that is being supplied to the passageways 22. Water 26 may be supplied to the chamber 24 from any suitable source of supply (not shown) through a supply pipe 28 in the wall of the chamber 24. The water is preferably under a predetermined regulated pressure to control the size and shape of the shot to be produced, as will be explained more fully hereinafter.

For the purpose of cooling and solidifying the metallic shot, a tank 16 partially filled with water is provided. The tank 16 is disposed directly beneath the shot ring 10 so as to receive the metallic shot when in its plastic state. In order that the water level in the tank 16 may remain constant, an overflow pipe 30 is provided. In practice, the water level in the tank 16 must be maintained at a constant value, otherwise the size of the metallic shot produced will vary.

Referring to Figs. 2 and 3, the passageways 22 are illustrated as being formed in tiers with the passageways 22 forming a single tier spaced close enough together to give a predetermined distribution of water in the center space of the shot ring 10. In the embodiment illustrated, the passageways 22 are preferably spaced 20 degrees apart with respect to a passageway in the same tier. In order to prevent too high a concentration of water at any one point and thereby cause a geysering effect upwardly from such a point, the passageways 22 are distributed in spaced tiers as illustrated in Fig. 3, the passageways 22 of each of the tiers being staggered with respect to the passageways 22 of the adjacent tiers. In a specific embodiment illustrated, three tiers of the staggered passageways 22 have been found to be satisfactory. In this embodiment, the three tiers of passageways 22 will provide a passageway 22 every 6 degrees and 40 minutes about the circumference of the hollow cylindrical wall member 20.

As illustrated, each of the passageways 22 in each tier is inclined downwardly and inwardly with respect to the member 20. The angle of inclination of the passageways is critical, being preferably between 20° and 60° with respect to the vertical as it is found that if the angle is larger than 60° then the jets of water impinge on one another in a manner to form a vertical column of water which may strike the bottom of the tundish 12, whereas if the angle is smaller than 20°, the jets of water are ineffective in breaking up the stream of molten metal into the uniformly sized shot desired. In practice, it is found that where the passageways 22 are disposed downwardly at an angle of 40° to the vertical the streams of water emitted from the passageways 22, as evidenced by the centerlines 32 extending from the passageways 22, impinge on the circumference of an imaginary circle 33 to effectively break up the stream of molten metal directed thereto into the required small particles.

No geysering of the water is obtained where the water jets strike the stream of molten metal in this manner.

While the jets of water are effective in breaking up the stream of molten metal into small particles, in order to impart a substantially spherical shape to the particles, the passageways 22 of each of the tiers are so drilled and positioned in the hollow cylindrical member 20 that the jets of water emerging from each tier impinge tangentially on the circumference of a  $\frac{1}{8}$  inch diameter imaginary circle centrally located with respect to the shot ring 10. By so positioning the passageways 22, the jets of water emerging therefrom effect a swirling or rotary motion of the water centrally located with respect to the shot ring 10. Each of the centrally located imaginary circles is not located in the plane formed by its associated tier of passageways 22 but rather is spaced a predetermined distance therefrom. It can be seen that with three spaced tiers of staggered water jets there will be three imaginary circles, the circumferences of which have jets of water impinging on them. As the molten metal strikes the jets of water, the jets break up the stream of metal and impart a rotary motion to the particles of molten metal to form substantially spherical shot. The rotary motion that is given the particles of molten metal is effected by having the jets of water formed by the passageways 22 impinge tangentially on the circumferences of their respective imaginary circles whereby the metal particles struck by one of the jets are carried toward the area of the imaginary circle, and as the metal particle passes from one impinging jet to the other, a rotary motion is imparted to the particle to impart a substantially spherical shape thereto.

In practice, it has been found desirable to provide a shot ring 10 whose cylindrical member 20 has an outside diameter of  $5\frac{3}{4}$  inches, a height of 3 inches, a wall thickness of  $\frac{3}{8}$  of an inch, and a distance of  $\frac{1}{2}$  inch between each of the tiers of passageways 22, the diameter of each of the passageways 22 being  $\frac{1}{8}$  of an inch with the passageways 22 disposed in the member 20 as described hereinbefore. A conical-shaped tundish 12 having an inside diameter of 14 inches at the top, a 3 inch inside diameter at the bottom, a height of 12 inches, a wall thickness of 1 inch at the top and  $1\frac{1}{2}$  inches at the bottom, and a diameter of  $\frac{3}{4}$  of an inch for the aperture 18 is satisfactory.

In practice, when using apparatus having the above dimensions, it is desirable to maintain the height of the metal in the tundish 12 at 2 inches to give a sufficient pressure head to the stream of metal flowing to the ring 10. With such a pressure head, the distance between the tundish 12 and the hollow shot ring 10 is maintained at 5 inches, and the distance between the hollow shot ring 10 and the level of the water in the tank 16 at 18 inches. In order to obtain proper results the water pressure should be maintained at 15 pounds per square inch and the pouring temperature of the molten metal between 1500° C. and 1525° C.

In operation, the molten metal is poured from the reservoir 14 into the clay-graphite tundish 12 to a height necessary to produce the desired pressure head. The tundish 12 is preferably preheated with a gas burner (not shown) prior to admitting the molten metal thereto to prevent chilling of the metal. The molten metal flows through the aperture or orifice 18 of the tundish

12 in a steady stream, as long as the pressure head is maintained, into the center space of the shot ring 10. When the stream of metal reaches the jets of water that emerge from the inclined and staggered passageways 22, the stream of molten metal is broken into particles and a rotary motion imparted thereto which forms the particles of plastic metal into substantially spherical shaped shot. The metallic shot thus produced is in a plastic state until it strikes the water in the tank 16. However, once the shot strikes the water and starts to fall to the bottom of the tank 16, it is so cooled that it solidifies to retain the substantially spherical shape imparted thereto. The shot may be removed from the tank 16 in a conventional manner.

The method embodying the teaching of this invention has many advantages. Among these are that the shot produced is more uniform in size and spherical in shape than that produced by prior known methods. This uniformity in size and spherical shape permits a more efficient removal of surface oxides during washing and blending.

From the operational point of view, the apparatus for carrying out the method of this invention possesses several advantages. The pouring time is appreciably decreased which permits maintaining a more nearly constant melt temperature and also aids in obtaining a more uniform size and shape of shot. Preheating of the tundish 12 is simplified since the tundish is movable and can be heated with a gas burner away from the reservoir 14 and the heated tundish 12 can then be positioned to receive the metal when the metal is ready to pour. In addition, the tundish 12, since it is not contaminated with slag, as was the formerly used V-shaped ceramic-lined trough, does not require any maintenance.

A still further advantage is that pouring is simplified considerably since no special precautions are required in order to maintain a constant stream of molten metal. This is automatically taken care of by keeping a predetermined head of molten metal in the tundish 12.

We claim as our invention:

1. In the method of making metallic shot, the steps comprising, providing a plurality of tiers of jets of water, each tier of water jets having an imaginary centrally located circle associated therewith, directing the jets of water of each tier so as to impinge tangentially on the circumference of their respective imaginary centrally located circle, combining the plurality of tiers of jets of water to simulate a cylinder of water rotating in one predetermined direction, and directing a stream of molten metal into the jets of water whereby the jets of water break the metal up into particles and carry the particles towards

the cylinder of rotating water, the jets imparting a rotary motion to the particles to produce substantially spherical shot therefrom as the particles pass from one to another of the impinging jets forming the cylinder of water.

5 2. In the method of making metallic shot, the steps comprising, providing a plurality of tiers of jets of water, each tier of water jets having an imaginary centrally located circle associated therewith, inclining the jets of water of each tier downwardly at an angle between 20° and 60° to the vertical, directing the jets of water of each tier so as to impinge tangentially on the circumference of their respective imaginary centrally located circle, combining the plurality of tiers of jets of water to simulate a cylinder of water rotating in one predetermined direction, and directing a stream of molten metal into the jets of water whereby the jets of water break the metal up into particles and carry the particles towards the cylinder of rotating water, the jets imparting a rotary motion to the particles to produce substantially spherical shot therefrom as the particles pass from one to another of the impinging jets forming the cylinder of water.

20 3. In the method of making metallic shot, the steps comprising, providing a plurality of tiers of jets of water, spacing the jets of water of any one tier not more than 20° apart, each tier of 30 water jets having an imaginary centrally located circle associated therewith, inclining the jets of water of each tier downwardly at an angle between 20° and 60° to the vertical, directing the jets of water of each tier so as to impinge tangentially on the circumference of their respective imaginary centrally located circle, combining the plurality of tiers of jets of water in vertically spaced relationship and staggering the jets of water of each tier with respect to the jets of water in the adjacent tier to simulate a cylinder of water rotating in one predetermined direction, and directing a stream of molten metal into the jets of water whereby the jets of water break the metal up into particles and carry the particles towards the cylinder of rotating water, the jets imparting a rotary motion to the particles to produce substantially spherical shot therefrom as the particles pass from one to another of the impinging jets forming the cylinder of water.

40 PAUL W. BEAMER.  
WILSON G. YOUNG, JR.

References Cited in the file of this patent

UNITED STATES PATENTS

| Number    | Name   | Date          |
|-----------|--------|---------------|
| 1,627,982 | Maguet | May 10, 1927  |
| 2,402,441 | Paddle | June 18, 1946 |
| 2,417,301 | Hayes  | Mar. 11, 1947 |